



US007910183B2

(12) **United States Patent**  
**Wu**

(10) **Patent No.:** **US 7,910,183 B2**  
(45) **Date of Patent:** **\*Mar. 22, 2011**

(54) **LAYERED INTERMEDIATE TRANSFER MEMBERS**

(75) Inventor: **Jin Wu**, Webster, NY (US)

(73) Assignee: **Xerox Corporation**, Norwalk, CT (US)

(\*) Notice: Subject to any disclaimer, the term of this patent is extended or adjusted under 35 U.S.C. 154(b) by 191 days.

This patent is subject to a terminal disclaimer.

(21) Appl. No.: **12/413,645**

(22) Filed: **Mar. 30, 2009**

(65) **Prior Publication Data**

US 2010/0247818 A1 Sep. 30, 2010

(51) **Int. Cl.**

**B41M 5/50** (2006.01)  
**G03G 15/16** (2006.01)

(52) **U.S. Cl.** ..... **428/32.51**; 428/195.1; 428/447; 428/473.5

(58) **Field of Classification Search** ..... None  
See application file for complete search history.

(56) **References Cited**

U.S. PATENT DOCUMENTS

5,487,707 A 1/1996 Sharf et al.  
6,318,223 B1 11/2001 Yu et al.

|                |         |                           |
|----------------|---------|---------------------------|
| 6,397,034 B1   | 5/2002  | Tarnawskyj et al.         |
| 6,440,515 B1   | 8/2002  | Thornton et al.           |
| 6,602,156 B2   | 8/2003  | Schlüter, Jr.             |
| 6,985,690 B2 * | 1/2006  | Odell et al. .... 399/333 |
| 7,031,647 B2   | 4/2006  | Mishra et al.             |
| 7,130,569 B2   | 10/2006 | Goodman et al.            |
| 7,139,519 B2   | 11/2006 | Darcy, III et al.         |

OTHER PUBLICATIONS

Jin Wu, U.S. Appl. No. 12/200,074 entitled Hydrophobic Carbon Black Intermediate Transfer Components, filed Aug. 28, 2008.

Jin Wu, U.S. Appl. No. 12/200,111 entitled Hydrophobic Polyetherimide/Polysiloxane Copolymer Intermediate Transfer Components, filed Aug. 28, 2008.

Jin Wu et al., U.S. Appl. No. 12/200,147 entitled Coated Seamed Transfer Member, filed Aug. 28, 2008.

Jin Wu et al., U.S. Appl. No. 12/200,179 entitled Coated Transfer Member, filed Aug. 28, 2008.

Jin Wu, U.S. Appl. No. 12/129,995 on Polyimide Intermediate Transfer Components, filed May 30, 2008.

Jin Wu, U.S. Appl. No. 12/181,354, on Core Shell Intermediate Transfer Components, filed Jul. 29, 2008.

Jin Wu, U.S. Appl. No. 12/181,409 on Treated Carbon Black Intermediate Transfer Components, filed Jul. 29, 2008.

\* cited by examiner

*Primary Examiner* — Bruce H Hess

(74) *Attorney, Agent, or Firm* — Oliff & Berridge, PLC

(57) **ABSTRACT**

An intermediate transfer media, such as a belt, that includes a first polyimide substrate layer and a second layer of a polyetherimide/polysiloxane polymer.

**30 Claims, No Drawings**

**LAYERED INTERMEDIATE TRANSFER  
MEMBERS**

**CROSS REFERENCE TO RELATED  
APPLICATIONS**

Copending U.S. application No. 12/413,627, U.S. Publication No. 20100248103, filed Mar. 30, 2009, entitled Resin Mixture Backing Layer Containing Photoconductor, the disclosure of which is totally incorporated herein by reference, illustrates a photoconductor comprising a substrate, an imaging layer thereon, and a backing layer located on a side of the substrate opposite the imaging layer wherein the outermost layer of the backing layer adjacent to the substrate is comprised of a glycoluril resin, and a polyol resin mixture.

Copending U.S. application No. 12/413,633, U.S. Publication No. 20100249322, filed Mar. 30, 2009, entitled Fluorinated Sulfonic Acid Polymer Grafted Polyaniline Containing Intermediate Transfer Members, the disclosure of which is totally incorporated herein by reference, illustrates an intermediate transfer member comprised of a substrate, and in contact therewith a polyaniline having grafted thereto a fluorinated sulfonic acid polymer.

Copending U.S. application No. 12/413,638, U.S. Publication No. 20100247918, filed Mar. 30, 2009, entitled Perfluoropolyether Polymer Grafted Polyaniline Containing Intermediate Transfer Members, the disclosure of which is totally incorporated herein by reference, illustrates an intermediate transfer member comprised of a substrate and in contact with the substrate a polyaniline grafted perfluoropolyether phosphoric acid polymer.

Copending U.S. application No. 12/413,642, U.S. Publication No. 20100247919, filed Mar. 30, 2009, entitled Fluorotelomer Grafted Polyaniline Containing Intermediate Transfer Members, the disclosure of which is totally incorporated herein by reference, illustrates An intermediate transfer member comprised of a substrate, and a layer comprised of polyaniline having grafted thereto a fluorotelomer.

Copending U.S. application No. 12/413,651, U.S. Publication No. 20100248106, filed Mar. 30, 2009, entitled Polyimide Polysiloxane Intermediate Transfer Members, the disclosure of which is totally incorporated herein by reference, illustrates an intermediate transfer member comprised of at least one of a polyimide/polyetherimide/polysiloxane, and a polyimide polysiloxane.

Copending U.S. Application No. 12/413,783, U.S. Publication No. 20100248107, filed Mar. 30, 2009, entitled Glycoluril Resin And Polyol Resin Members, the disclosure of which is totally incorporated herein by reference, illustrates a process which comprises providing a flexible belt having at least one welded seam extending from one parallel edge to the other parallel edge, the welded seam having a rough seam region comprising an overlap of two opposite edges; contacting the rough seam region with a heat and pressure applying tool; and smoothing out the rough seam region with heat and pressure applied by the heat and pressure applying tool to produce a flexible belt having a smooth welded seam, and subsequently coating the seam with a resin mixture of a glycoluril resin and a polyol resin.

Copending U.S. application No. 12/413,795, U.S. Publication No. 20100248108, filed Mar. 30, 2009, entitled Glycoluril Resin And Polyol Resin Dual Members, the disclosure of which is totally incorporated herein by reference, illustrates a process which comprises providing a flexible belt having at least one welded seam extending from one parallel edge to the other parallel edge of the coating, the welded seam having a rough seam region comprising an overlap of two opposite edges; contacting the rough seam region with a heat and pressure applying tool; and smoothing out the rough

seam region with heat and pressure applied by the heat and pressure applying tool, and subsequently coating the belt with a resin mixture of a glycoluril resin and a polyol resin.

Copending U.S. application No. 12/413,832, U.S. Publication No. 20100248104, filed Mar. 30, 2009, entitled Polyaniline Dialkylsulfate Complexes Containing Intermediate Transfer Members, the disclosure of which is totally incorporated herein by reference, illustrates an intermediate transfer member comprised of a polyaniline dialkylsulfate complex.

10 Copending U.S. Application No. 12/413,852, U.S. Publication No. 20100248102, filed Mar. 30, 2009, entitled Crosslinked Resin Mixture Backing Layer Containing Photoconductor, the disclosure of which is totally incorporated herein by reference, illustrates a photoconductor comprising a substrate, an imaging layer thereon, and a backing layer located on a side of the substrate opposite the imaging layer wherein the outermost layer of the backing layer adjacent to the substrate is comprised of a mixture of glycoluril resin and a polyacetal resin mixture.

15 20 Illustrated in U.S. application Ser. No. 12/200,074, U.S. Publication No. 20100055463, entitled Hydrophobic Carbon Black Intermediate Transfer Components, filed Aug. 28, 2008, the disclosure of which is totally incorporated herein by reference, is an intermediate transfer member comprised of a substrate comprising a carbon black surface treated with a poly(fluoroalkyl acrylate).

25 30 Illustrated in U.S. application Ser. No. 12/200,111, U.S. Publication No. 20100055445, entitled Hydrophobic Polyetherimide/Polysiloxane Copolymer Intermediate Transfer Components, filed Aug. 28, 2008, is an intermediate transfer member comprised of a substrate comprising a polyetherimide polysiloxane copolymer.

35 40 Illustrated in U.S. application Ser. No. 12/200,147, U.S. Publication No. 20100055328, entitled Coated Seamed Transfer Member, filed Aug. 28, 2008, is a process which comprises providing a flexible belt having a welded seam extending from one parallel edge to the other parallel edge, the welded seam having a rough seam region comprising an overlap of two opposite edges; contacting the rough seam region with a heat and pressure applying tool; and smoothing out the rough seam region with heat and pressure applied by the heat and pressure applying tool to produce a flexible belt having a smooth welded seam, and subsequently coating the seam with a crosslinked acrylic resin.

45 50 Illustrated in U.S. application Ser. No. 12/200,179, U.S. Publication No. 20100051171, entitled Coated Transfer Member, filed Aug. 28, 2008, is a process which comprises providing a flexible belt having a welded seam extending from one parallel edge to the other parallel edge, the welded seam having a rough seam region comprising an overlap of two opposite edges; contacting the rough seam region with a heat and pressure applying tool; and smoothing out the rough seam region with heat and pressure applied by the heat and pressure applying tool to produce a flexible belt having a smooth welded seam, and subsequently coating the belt with a crosslinked acrylic resin.

55 60 Illustrated in U.S. application Ser. No. 12/129,995, U.S. Publication No. 20090297232, filed May 30, 2008, entitled Polyimide Intermediate Transfer Components, the disclosure of which is totally incorporated herein by reference, is an intermediate transfer belt comprised of a substrate comprising a polyimide and a conductive component wherein the polyimide is cured at a temperature of for example, from about 175° C. to about 290° C. over a period of time of from about 10 minutes to about 120 minutes.

65 Illustrated in U.S. application Ser. No. 12/181,354, U.S. Publication 20100028700, filed Jul. 29, 2008, entitled Core Shell Intermediate Transfer Components, the disclosure of which is totally incorporated herein by reference, is an intermediate transfer belt comprised of a substrate comprising a conductive core shell component.

Illustrated in U.S. application Ser. No. 12/181,409, now U.S. Pat. No. 7,738,824, filed Jul. 29, 2008, entitled Treated Carbon Black Intermediate Transfer Components, the disclosure of which is totally incorporated herein by reference, is an intermediate transfer members comprised of a substrate comprising a poly(vinylalkoxysilane) surface treated carbon black.

## BACKGROUND

Disclosed are intermediate transfer members, and more specifically, intermediate transfer members useful in transferring a developed image in an electrostatographic, for example xerographic, including digital, image on image, and the like, machines or apparatuses and printers. In embodiments, there are selected intermediate transfer members comprised of a first polyimide layer and a second polyetherimide-b-polysiloxane layer, and more specifically, where the economical polyetherimide-b-polysiloxane layer is in full contact with the polyimide layer and where there can be included in at least one of the first and second layers a conductive component. A number of advantages are associated with the intermediate transfer members of the present disclosure, such as excellent mechanical characteristics, robustness, consistent, and excellent surface resistivities, and acceptable adhesion properties, especially when there is included in the intermediate transfer member an adhesive layer; excellent maintained conductivity or resistivity for extended time periods; dimensional stability; ITB humidity insensitivity for extended time periods; excellent dispersability in a polymeric solution; low and acceptable surface friction characteristics; and minimum or substantially no peeling or separation of the layers.

One specific advantage of the disclosed two-layer ITB is its low surface energy, for example, a contact angle of about 100° (degrees) for the block copolymer as compared to about 50° for the polyimide layer, which advantage is of value with regard to improved toner transfer and cleaning, where in embodiments the top layer functions primarily to obtain high fidelity transfer in view of its low surface energy, while the base polyimide layer provides reliable mechanical strength.

In aspects thereof, the present disclosure relates to a multi-layer intermediate transfer layer, such as a belt (ITB) comprised of a polyimide base layer and a polyetherimide-b-polysiloxane block copolymer top layer, and where each layer further includes a conductive component, and an optional adhesive layer situated between the two layers, and which layered member can be prepared by known solution casting methods and known extrusion molded processes with the optional adhesive layer can be generated and applied by known spray coating and flow coating processes.

Furthermore, disclosed herein is a hydrophobic intermediate transfer member having a surface resistivity of from about 10<sup>7</sup> to about 10<sup>14</sup> ohm/sq. or from about 10<sup>9</sup> to about 10<sup>12</sup> ohm/sq. and a bulk resistivity of from about 10<sup>7</sup> to about 10<sup>14</sup> ohm/sq. or from about 10<sup>9</sup> to about 10<sup>12</sup> ohm cm.

The ITB member comprised of the disclosed hydrophobic polyetherimide-b-polysiloxane block copolymer is, for example, hydrophobic, such as an about 50 percent more hydrophobic as determined by an about 50° higher contact angle as compared to an ITB that does not contain the polyetherimide-b-polysiloxane block copolymer. In addition, primarily because of the ITB water repelling properties determined, for example, by accelerated aging experiments at 80° F./80 percent humidity, for four weeks, the surface resistivity of the disclosed hydrophobic ITB member remained

unchanged, while that of the a similar comparative member which is free of the polyetherimide-b-polysiloxane varied.

In a typical electrostatographic reproducing apparatus, a light image of an original to be copied is recorded in the form of an electrostatic latent image upon a photosensitive member, and the latent image is subsequently rendered visible by the application of electroscopic thermoplastic resin particles and colorant. Generally, the electrostatic latent image is developed by contacting it with a developer mixture comprised of a dry developer mixture, which usually comprises carrier granules having toner particles adhering triboelectrically thereto, or a liquid developer material, which may include a liquid carrier having toner particles dispersed therein. The developer material is advanced into contact with the electrostatic latent image, and the toner particles are deposited thereon in image configuration. Subsequently, the developed image is transferred to a copy sheet. It is advantageous to transfer the developed image to a coated intermediate transfer web, belt or component, and subsequently transfer with a high transfer efficiency the developed image from the intermediate transfer member to a permanent substrate. The toner image is subsequently usually fixed or fused upon a support, which may be the photosensitive member itself, or other support sheet such as plain paper.

In electrostatographic printing machines wherein the toner image is electrostatically transferred by a potential difference between the imaging member and the intermediate transfer member, the transfer of the toner particles to the intermediate transfer member, and the retention thereof should be substantially complete so that the image ultimately transferred to the image receiving substrate will have a high resolution. Substantially about 100 percent toner transfer occurs when most or all of the toner particles comprising the image are transferred, and little residual toner remains on the surface from which the image was transferred.

Intermediate transfer members possess a number of advantages, such as enabling high throughput at modest process speeds; improving registration of the final color toner image in color systems using synchronous development of one or more component colors, and using one or more transfer stations; and increasing the number of substrates that can be selected. However, a disadvantage of using an intermediate transfer member is that a plurality of transfer operations is usually needed allowing for the possibility of charge exchange occurring between toner particles, and the transfer member which ultimately can lead to less than complete toner transfer, resulting in low resolution images on the image receiving substrate, and image deterioration. When the image is in color, the image can additionally suffer from color shifting and color deterioration.

Attempts at controlling the resistivity of intermediate transfer members by, for example, adding conductive fillers, such as ionic additives and/or carbon black to the outer layer, are disclosed in U.S. Pat. No. 6,397,034 which describes the use of fluorinated carbon filler in a polyimide intermediate transfer member layer. However, there can be problems associated with the use of such fillers in that undissolved particles frequently bloom or migrate to the surface of the fluorinated polymer and cause imperfections to the polymer, thereby causing nonuniform resistivity, which in turn causes poor antistatic properties and poor mechanical strength characteristics. Also, ionic additives on the ITB surface may interfere with toner release. Furthermore, bubbles may appear in the polymer, some of which can only be seen with the aid of a microscope, and others of which are large enough to be observed with the naked eye resulting in poor or nonuniform electrical properties and poor mechanical properties.

In addition, the ionic additives themselves are sensitive to changes in temperature, humidity, and operating time. These sensitivities often limit the resistivity range. For example, the resistivity usually decreases by up to two orders of magnitude or more as the humidity increases from about 20 percent to 80 percent relative humidity. This effect limits the operational or process latitude.

Moreover, ion transfer can also occur in these systems. The transfer of ions leads to charge exchanges and insufficient transfers, which in turn causes low image resolution and image deterioration, thereby adversely affecting the copy quality. In color systems, additional adverse results include color shifting and color deterioration. Ion transfer also increases the resistivity of the polymer member after repetitive use. This can limit the process and operational latitude, and eventually the ion filled polymer member will be unusable.

Therefore, it is desired to provide an intermediate transfer member with a number of the advantages illustrated herein such as excellent mechanical, and humidity insensitivity characteristics permitting high copy quality where developed images with minimal resolution issues can be obtained. It is also desired to provide a weldable intermediate transfer belt that may not, but could, have puzzle cut seams, and instead, has a weldable seam, thereby providing a belt that can be manufactured without labor intensive steps, such as manually piecing together the puzzle cut seam with fingers, and without the lengthy high temperature and high humidity conditioning steps.

A number of the known ITB formulations apply carbon black or polyaniline as the conductive species, however, this has some limitations. For example, polyaniline is readily oxidized and results in loss of conductivity, its thermal stability is usually limited to about 200° C., and it begins to lose its conductivity at above 200° C. Also, it can be difficult to prepare carbon black based ITBs with consistent resistivity because the required loadings reside on the vertical part of the percolation curve. The amount of carbon black and how carbon black is processed (primary particle size and aggregate size) are of value for conductivity and for the manufacturing of intermediate belts.

#### REFERENCES

Illustrated in U.S. Pat. No. 7,031,647 is an imageable seamed belt containing a lignin sulfonic acid doped polyaniline.

Illustrated in U.S. Pat. No. 7,139,519 is an intermediate transfer belt, comprising a belt substrate comprising primarily at least one polyimide polymer; and a welded seam.

Illustrated in U.S. Pat. No. 7,130,569 is a weldable intermediate transfer belt comprising a substrate comprising a homogeneous composition comprising a polyaniline in an amount of, for example, from about 2 to about 25 percent by weight of total solids, and a thermoplastic polyimide present in an amount of from about 75 to about 98 percent by weight of total solids, wherein the polyaniline has a particle size of, for example, from about 0.5 to about 5 microns.

Puzzle cut seam members are disclosed in U.S. Pat. Nos. 5,487,707; 6,318,223, and 6,440,515.

Illustrated in U.S. Pat. No. 6,602,156 is a polyaniline filled polyimide puzzle cut seamed belt, however, the manufacture of a puzzle cut seamed belt is labor intensive and costly, and the puzzle cut seam, in embodiments, is sometimes weak. The manufacturing process for a puzzle cut seamed belt usually involves a lengthy in time high temperature and high humidity conditioning step. For the conditioning step, each individual belt is rough cut, rolled up, and placed in a conditioning chamber that is environmentally controlled at about 45° C. and about 85 percent relative humidity, for approximately 20 hours. To prevent or minimize condensation and watermarks, the puzzle cut seamed transfer belt resulting is permitted to remain in the conditioning chamber for a suitable period of time, such as 3 hours. The conditioning of the transfer belt renders it difficult to automate the manufacturing thereof, and the absence of such conditioning may adversely impact the belts electrical properties, which in turn results in poor image quality.

#### SUMMARY

In embodiments, there is disclosed an intermediate transfer member comprised of a polyimide substrate, and thereover a polyetherimide/polysiloxane layer; a transfer media comprised of a polyimide first supporting substrate layer and thereover a second layer comprised of a polyetherimide-block-polysiloxane copolymer, an adhesive layer situated between the first layer and the second layer, and wherein at least one of the first layer and the second layer further contain a known conductive component like carbon black, a polyaniline, and the like; an intermediate transfer belt comprised of a polyimide substrate layer, and thereover a layer comprised of a polyetherimide/polysiloxane copolymer; and wherein at least one of the substrate layer and the copolymer layer further contains a conductive component, and wherein the polyetherimidepolysiloxane copolymer is represented by



wherein the substrate is of a thickness of from about 70 to about 125 microns, and the polyetherimide-b-polysiloxane copolymer in the form of a layer is of a thickness of from about 5 to about 15 microns, and the polyetherimide-b-polysiloxane copolymer possesses a weight average molecular weight of from about 100,000 to about 200,000, wherein the weight percent of thereof of the polysiloxane in the copolymer is from about 20 to about 75, and wherein the total of the components in the copolymer layer is about 100 percent; an intermediate transfer member, such as an intermediate belt, comprised of a substrate comprising, for example, a polyimide, and thereover a layer comprised of a polyetherimide/polysiloxane polymer like a polyetherimide-b-polysiloxane block copolymer; an intermediate transfer member comprised primarily of a polyetherimide-b-polysiloxane copolymer formed by reacting pyromellitic acid with diaminodiphenylether and an aminopropyl-terminated

medium comprising a photoconductor surface with an electrostatic latent image thereon; a development source to apply toner to the photoconductor, and to develop the electrostatic latent image, followed by transfer of the developed image to a substrate like paper or other suitable material like plastic, followed by fixing the developed image to the substrate which fixing can be accomplished by heat.

Specific examples of polysiloxane/polyetherimides that may be selected for the intermediate transfer member, inclusive of an intermediate transfer belt, include a number of known polymers such as a polysiloxane/polyetherimide block copolymer available as ULTEM® STM1500 ( $T_g=168^\circ C.$ ); ULTEM® STM1600 ( $T_g=195^\circ C.$ ); and ULTEM® STM1700 ( $T_g=200^\circ C.$ ), commercially available from Sabic Innovative Plastics. The chemical structure of ULTEM® STM1500 can be, it is believed, represented by the following



polydimethylsiloxane; reacting biphenyltetracarboxylic acid and pyromellitic acid with p-phenylenediamine, diaminodiphenylether and an aminopropyl-terminated polydimethylsiloxane; or by reacting pyromellitic dianhydride and a benzophenone tetracarboxylic dianhydride copolymeric acid with 2,2-bis[4-(8-aminophenoxy)phenoxy]-hexafluoropropane and an aminopropyl-terminated polydimethylsiloxane.

Furthermore, there is disclosed an intermediate transfer member comprised of a polyimide supporting substrate, a polyetherimide-b-polysiloxane block copolymer layer thereover, and where each layer contains a conductive component such as a polyaniline, carbon black, a metal oxide, and the like; an apparatus for forming images on a recording medium comprising a charge retentive surface to receive an electrostatic latent image thereon; a development component to apply toner to the charge retentive surface, such as a photoconductor, to develop the electrostatic latent image, and to form a developed image on the charge retentive surface; and an intermediate transfer media that functions to transfer the developed image from the charge retentive surface to a substrate, wherein the intermediate transfer media is comprised of a polyimide substrate, and in contact with the substrate a polyetherimide polysiloxane polymer layer.

In addition, the present disclosure provides, in embodiments, an apparatus for forming images on a recording

The weight average molecular weight ( $M_w$ ) of the polysiloxane/polyetherimide can vary, for example, from about 5,000 to about 1,000,000, from about 20,000 to about 500,000, from about 50,000 to about 300,000, and from about 75,000 to about 175,000, and the like, wherein the weight percent of the polysiloxane block in the block copolymer is, for example, from about 5 to about 95, from about 10 to about 75, from about 15 to about 50, from about 20 to about 40, and other suitable percentages, and wherein the total of the components in the copolymer is about 100 percent.

A specific polysiloxane/polyetherimide polymer and copolymer, which is available from Sabic Innovative Plastics, can be prepared, for example, by reacting 2,2-bis(2,3-dicarboxyphenoxyphenol)propane dianhydride with metaphenyl-diamine, and an aminopropyl-terminated D10 polydimethylsiloxane. D10 refers to a decamer of the siloxane as represented by  $-\text{Si}(\text{CH}_3)_2\text{O}-$ , and is a specific example of a ULTEM material illustrated herein.

Examples of specific selected first or supporting layer thermoplastic polyimides are KAPTON® KJ, commercially available from E.I. DuPont, Wilmington, Del., as represented by



wherein x is equal to 2; y is equal to 2; m and n are from about 10 to about 300; and IMIDEX®, commercially available from West Lake Plastic Company, as represented by

10 RC-5069, RC-5097, RC-5053, and RK-692, all commercially available from Industrial Summit Technology Corporation, Parlin, N.J.; RP-46 and RP-50, both commercially



25 wherein z is equal to 1, and q is from about 10 to about 300.

A number of the thermosetting polyimides selected as the first supporting layer, in embodiments, illustrated in the appropriate copending applications recited herein can be cured at suitable temperatures, and more specifically, from about 180° C. to about 260° C. over a short period of time, such as, for example, from about 10 to about 120 minutes, and from about 20 to about 60 minutes; possess, for example, a number average molecular weight of from about 5,000 to about 500,000, or from about 10,000 to about 100,000, and a weight average molecular weight of from about 50,000 to about 5,000,000, or from about 100,000 to about 1,000,000; thermosetting polyimide precursors that are cured at higher temperatures (above 300° C.) than the VTEC™ PI polyimide precursors, and which precursors include, for example, PYRE-M.L® RC-5019, RC-5057, RC-5069, RC-5097, RC-5053, and RK-692, all commercially available from Industrial Summit Technology Corporation, Parlin, N.J.; RP-46 and RP-50, both commercially available from Unitech LLC, Hampton, Va.; DURIMIDE® 100 commercially available from FUJIFILM Electronic Materials U.S.A., Inc., North Kingstown, R.I.; and KAPTON® HN, VN and FN, all commercially available from E.I. DuPont, Wilmington, Del., in amounts of, for example, of from about 70 to about 97, or from about 80 to about 95 weight percent of the intermediate transfer member.

50 Examples of thermosetting polyimides that can be incorporated into the first layer of the intermediate transfer member include known low temperature and rapidly cured polyimide polymers, such as VTEC™ PI 1388, 080-051, 851, 302, 203, 201, and PETI-5, all available from Richard Blaine International, Incorporated, Reading, Pa. These thermosetting polyimides can be cured at temperatures of from about 180° C. to about 260° C. over a short period of time, such as from about 10 to about 120 minutes, or from about 20 to about 60 minutes; possess a number average molecular weight of from about 5,000 to about 500,000, or from about 10,000 to about 100,000, and a weight average molecular weight of from about 50,000 to about 5,000,000, or from about 100,000 to about 1,000,000. Other thermosetting polyimides that can be selected for the ITM or ITB, and cured at temperatures of above 300° C. include PYRE M.L® RC-5019, RC 5057,

available from Unitech LLC, Hampton, Va.; DURIMIDE® 100 commercially available from FUJIFILM Electronic Materials U.S.A., Inc., North Kingstown, R.I.; and KAPTON® HN, VN and FN, all commercially available from E.I. DuPont, Wilmington, Del.

35 Suitable supporting substrate polyimides include those formed from various diamines and dianhydrides, such as poly(amidimide), polyetherimide, polysiloxane polyetherimide block copolymer, and the like. Preferred polyimides include aromatic polyimides such as those formed by the reacting pyromellitic acid and diaminodiphenylether, or by imidization of copolymeric acids such as biphenyltetracarboxylic acid and pyromellitic acid with two aromatic diamines such as p-phenylenediamine and diaminodiphenylether. Another suitable polyimide includes pyromellitic dianhydride and benzophenone tetracarboxylic dianhydride copolymeric acids reacted with 2,2-bis[4-(8-aminophenoxy) phenoxy]-hexafluoropropane. Other suitable aromatic polyimides include those containing 1,2,1',2'-biphenyltetracarboximide and para-phenylene groups, and those having biphenyltetracarboximide functionality with diphenylether end spacer characterizations. Mixtures of polyimides can also be used.

40 The conductive material, such as a carbon black, a metal oxide or polyaniline, is present in at least one layer of the intermediate transfer member in, for example, an amount of from about 1 to about 30 weight percent, from about 3 to about 20 weight percent, or preferably from about 5 to about 15 weight percent.

45 Carbon black surface groups can be formed by oxidation with an acid or with ozone, and where there is absorbed or chemisorbed oxygen groups from, for example, carboxylates, phenols, and the like. The carbon surface is essentially inert to most organic reaction chemistry except primarily for oxidative processes and free radical reactions.

50 The conductivity of carbon black is dependent on surface area and its structure primarily. Generally, the higher surface area and the higher structure, the more conductive the carbon black. Surface area is measured by the B.E.T. nitrogen surface area per unit weight of carbon black, and is the measurement of the primary particle size. Structure is a complex property that refers to the morphology of the primary aggregates of

## 11

carbon black. It is a measure of both the number of primary particles comprising primary aggregates, and the manner in which they are "fused" together. High structure carbon blacks are characterized by aggregates comprised of many primary particles with considerable "branching" and "chaining", while low structure carbon blacks are characterized by compact aggregates comprised of fewer primary particles. Structure is measured by dibutyl phthalate (DBP) absorption by the voids within carbon blacks. The higher the structure, the more the voids, and the higher the DBP absorption.

Examples of carbon blacks selected as the conductive component include VULCAN® carbon blacks, REGAL® carbon blacks, and BLACK PEARLS® carbon blacks available from Cabot Corporation. Specific examples of conductive carbon blacks are BLACK PEARLS® 1000 (B.E.T. surface area=343 m<sup>2</sup>/g, DBP absorption=105 ml/g), BLACK PEARLS® 880 (B.E.T. surface area=240 m<sup>2</sup>/g, DBP absorption=106 ml/g), BLACK PEARLS® 800 (B.E.T. surface area=230 m<sup>2</sup>/g, DBP absorption=68 ml/g), BLACK PEARLS® L (B.E.T. surface area=138 m<sup>2</sup>/g, DBP absorption=61 ml/g), BLACK PEARLS® 570 (B.E.T. surface area=110 m<sup>2</sup>/g, DBP absorption=114 ml/g), BLACK PEARLS® 170 (B.E.T. surface area=35 m<sup>2</sup>/g, DBP absorption=122 ml/g), VULCAN® XC72 (B.E.T. surface area=254 m<sup>2</sup>/g, DBP absorption=176 ml/g), VULCAN® XC72R (fluffy form of VULCAN® XC72), VULCAN® XC605, VULCAN® XC305, REGAL® 660 (B.E.T. surface area=112 m<sup>2</sup>/g, DBP absorption=59 ml/g), REGAL® 400 (B.E.T. surface area=96 m<sup>2</sup>/g, DBP absorption=69 ml/g), and REGAL® 330 (B.E.T. surface area=94 m<sup>2</sup>/g, DBP absorption=71 ml/g).

As illustrated herein, the carbon black is usually formed into a dispersion, such as a blend of the polyetherimide/polysiloxane copolymer, and a blend of the polyimide. With proper milling processes, uniform dispersions can be obtained, and then coated on glass plates using a draw bar coating method. The resulting individual films can be dried at high temperatures, such as from about 100° C. to about 400° C., for a suitable period of time, such as from about 20 to about 180 minutes, while remaining on the separate glass plates. After drying and cooling to room temperature, about 23° C. to about 25° C., the films on the glass plates can be immersed into water overnight, about 18 to 23 hours, and subsequently the 50 to 150 micron thick films can be released from the glass to form a functional intermediate transfer member.

In embodiments, the polyaniline component has a relatively small particle size of from about 0.5 to about 5, from about 1.1 to about 2.3, from about 1.2 to about 2, from about 1.5 to about 1.9, or about 1.7 microns. Specific examples of polyanilines selected for the transfer member, such as an ITB, are PANIPOL™ F, commercially available from Panipol Oy, Finland.

Adhesive layer components, and which layer is usually situated between the supporting substrate and the top poly-etherimide-b-polysiloxane block copolymer thereover, are a number of epoxy, urethane, silicone, polyester, and the like. Generally, the adhesive layer is a solventless layer that is materials that are liquid at room temperature (about 25° C.) and are able to crosslink to an elastic or rigid film to adhere at least two materials together. Specific examples include 100 percent solids adhesives including polyurethane adhesives from Lord Corporation, Erie, Pa., such as TYCEL® 7924 (viscosity from about 1,400 to about 2,000 cps), TYCEL® 7975 (viscosity from about 1,200 to about 1,600 cps) and TYCEL® 7276. The viscosity range of the adhesives is from about 1,200 to about 2,000 cps. The solventless adhesives can

## 12

be activated with either heat, room temperature curing, moisture curing, ultraviolet radiation, infrared radiation, electron beam curing, or any other known technique. The thickness of the adhesive layer is usually less than 100 nanometers, and more specifically, as illustrated hereinafter.

The thickness of each layer of the intermediate transfer member can vary and is not limited to any specific value. In specific embodiments, the substrate layer thickness is, for example, from about 20 to about 300, from about 30 to about 100, from about 75 to about 150, from about 50 to about 100 microns, while the thickness of the top polyetherimide-b-polysiloxane block copolymer is, for example, from about 1 to about 70 microns, from about 1 to about 40 microns, from about 1 to about 30 microns, and from about 10 to about 30 microns. The adhesive layer thickness is, for example, from about 1 to about 100 nanometers, from about 5 to about 75 nanometers, or from about 50 to about 100 nanometers.

The disclosed intermediate transfer members are in, embodiments, weldable, that is the seam of the member like 20 a belt is weldable, and more specifically, may be ultrasonically welded to produce a seam. The surface resistivity of the disclosed intermediate transfer member is, for example, from about 10<sup>9</sup> to about 10<sup>13</sup>, or from about 10<sup>10</sup> to about 10<sup>12</sup> ohm/sq. The sheet resistivity of the intermediate transfer 25 weldable member is, for example, from about 10<sup>9</sup> to about 10<sup>13</sup>, or from about 10<sup>10</sup> to about 10<sup>12</sup> ohm/sq.

The intermediate transfer members illustrated herein like intermediate transfer belts, can be selected for a number of printing, and copying systems, inclusive of xerographic printing. For example, the disclosed intermediate transfer members can be incorporated into a multi-imaging system where 30 each image being transferred is formed on the imaging or photoconductive drum at an image forming station, wherein each of these images is then developed at a developing station, 35 and transferred to the intermediate transfer member. The images may be formed on the photoconductor and developed sequentially, and then transferred to the intermediate transfer member. In an alternative method, each image may be formed on the photoconductor or photoreceptor drum, developed, 40 and transferred in registration to the intermediate transfer member. In an embodiment, the multi-image system is a color copying system, wherein each color of an image being copied is formed on the photoreceptor drum, developed, and transferred to the intermediate transfer member.

After the toner latent image has been transferred from the photoreceptor drum to the intermediate transfer member, the intermediate transfer member may be contacted under heat and pressure with an image receiving substrate such as paper. The toner image on the intermediate transfer member is then transferred and fixed, in image configuration, to the substrate 45 such as paper.

The intermediate transfer member present in the imaging systems illustrated herein, and other known imaging and printing systems, may be in the configuration of a sheet, a 50 web, a belt, including an endless belt, an endless seamed flexible belt, and an endless seamed flexible belt; a roller, a film, a foil, a strip, a coil, a cylinder, a drum, an endless strip, and a circular disc. The intermediate transfer member can be comprised of a single layer or it can be comprised of several 55 layers, such as from about 2 to about 5 layers. In embodiments, the intermediate transfer member further includes an outer release layer.

Release layer examples situated on and in contact with the second layer include low surface energy materials, such as 60 TEFLON®-like materials including fluorinated ethylene propylene copolymer (FEP), polytetrafluoroethylene (PTFE), polyfluoroalkoxy polytetrafluoroethylene (PFA TEFLON®)

13

and other TEFILON®-like materials; silicone materials such as fluorosilicones and silicone rubbers such as Silicone Rubber 552, available from Sampson Coatings, Richmond, Va., (polydimethyl siloxane/dibutyl tin diacetate, 0.45 gram DBTDA per 100 grams polydimethyl siloxane rubber mixture, with a molecular weight  $M_w$  of approximately 3,500); and fluoroelastomers such as those sold as VITON® such as copolymers and terpolymers of vinylidenefluoride, hexafluoropropylene, and tetrafluoroethylene, which are known commercially under various designations as VITON A®, VITON E®, VITON E60C®, VITON E45®, VITON E430®, VITON B910®, VITON GH®, VITON B50®, VITON E45®, and VITON GF®. The VITON® designation is a Trademark of E.I. DuPont de Nemours, Inc. Two known fluoroelastomers are comprised of (1) a class of copolymers of vinylidenefluoride, hexafluoropropylene, and tetrafluoroethylene, known commercially as VITON A®, (2) a class of terpolymers of vinylidenefluoride, hexafluoropropylene and tetrafluoroethylene known commercially as VITON B®, and (3) a class of tetrapolymers of vinylidenefluoride, hexafluoropropylene, tetrafluoroethylene, and a cure site monomer such as VITON GF® having 35 mole percent of vinylidenefluoride, 34 mole percent of hexafluoropropylene, and 29 mole percent of tetrafluoroethylene with 2 percent cure site monomer. The cure site monomer can be those available from DuPont such as 4-bromoperfluorobutene-1, 1,1-dihydro-4-bromoperfluorobutene-1, 3-bromoperfluoropropene-1, 1,1-dihydro-3-bromoperfluoropropene-1, or any other suitable known commercially available cure site monomer.

The layer or layers may be deposited on the substrate by known coating processes. Known methods for forming the outer layer(s) on the substrate film, such as dipping, spraying, such as by multiple spray applications of very thin films, casting, flow-coating, web-coating, roll-coating, extrusion, molding, or the like, can be used. It is preferred to deposit the layers by spraying such as by multiple spray applications of very thin films, casting, by web coating, by flow-coating, and most preferably by laminating.

The circumference of the intermediate transfer member, especially as it is applicable to a film or a belt configuration, is, for example, from about 250 to about 2,500 millimeters, from about 1,500 to about 3,000 millimeters, or from about 2,000 to about 2,200 millimeters with a corresponding width of, for example, from about 100 to about 1,000 millimeters, from about 200 to about 500 millimeters, or from about 300 to about 400 millimeters.

Specific embodiments will now be described in detail. These examples are intended to be illustrative, and are not limited to the materials, conditions, or process parameters set forth in these embodiments. All parts are percentages by weight of total solids unless otherwise indicated.

#### COMPARATIVE EXAMPLE 1

A one-layer polyimide intermediate transfer belt (ITB) member was prepared as follows.

One gram of PANIPOL® F, a hydrochloric acid doped emeraldine salt obtained from Panipol Oy (Porvoo Finland), was mixed with 28.3 grams of the polyamic acid solution, VTECTM PI 1388 (polyimide, 20 weight percent solids in NMP, obtained from Richard Blaine International, Incorporated). By ball milling this mixture with 2 millimeter stainless shot with an Attritor for 2 hours, a uniform dispersion of the aforementioned components was obtained.

The dispersion obtained above was then coated on a glass plate using a known draw bar coating method. Subsequently, the film obtained was dried at 100° C. for 20 minutes, and then

14

204° C. for an additional 20 minutes while remaining on the glass plate. After drying and cooling for about 3 hours to room temperature, the film on the glass plate was immersed into water overnight, about 23 hours, and a 80 micron thick freestanding film was released from the glass automatically resulting in an intermediate transfer member comprised of the above polyaniline/polyimide with a ratio by weight of 15/85.

#### EXAMPLE I

10 A two-layer intermediate transfer belt (ITB) member with a polyimide base layer and a polyetherimide-b-polysiloxane top layer was prepared as follows.

15 One gram of PANIPOL® F, a hydrochloric acid doped emeraldine salt, obtained from Panipol Oy (Porvoo Finland), was mixed with 28.3 grams of the polyamic acid solution, VTECTM PI 1388 (polyimide, 20 weight percent solids in NMP, obtained from Richard Blaine International, Incorporated). By ball milling this mixture with 2 millimeter stainless shot with an Attritor for 2 hours, a uniform dispersion was obtained. The dispersion was then coated on a glass plate using a known draw bar coating method. Subsequently, the film obtained was dried at 100° C. for 20 minutes, and then 20 204° C. for an additional 20 minutes while remaining on the glass plate.

25 Thereafter, one gram of PANIPOL® F, a hydrochloric acid doped emeraldine salt, obtained from Panipol Oy (Porvoo Finland), was mixed with 9 grams of ULTEM® STM1500 (Tg=168° C.), a polyetherimide-b-polysiloxane block 30 copolymer commercially available from Sabic Innovative Plastics, and 100 grams of methylene chloride. By ball milling this mixture with 2 millimeter stainless shot overnight, 23 hours, a uniform dispersion was obtained. The resulting dispersion was then coated on the above polyaniline/polyimide base supporting layer present on the glass plate, and dried at 120° C. for 5 minutes.

35 The resulting two-layer film on the glass was then immersed into water overnight, about 23 hours, and the freestanding film was released from the glass resulting in a two-layer intermediate transfer member with a 80 micron thick 40 polyaniline/polyimide base layer with a ratio by weight of 15 polyaniline/85 polyimide, and a 20 micron thick polyaniline/polyetherimide-b-polysiloxane top layer with a ratio by weight of 10 polyaniline/90 polyetherimide-b-polysiloxane.

#### EXAMPLE II

45 A three-layer intermediate transfer belt (ITB) member with a polyimide base layer, a solventless adhesive layer, and a polyetherimide-b-polysiloxane top layer is prepared by 50 repeating the process of Example I except that a solventless adhesive layer is incorporated between the polyimide base layer and the polyetherimide-b-polysiloxane top layer.

The solventless adhesive, TYCEL® 7975-A (adhesive) and 55 7276 (curing agent), both obtained from Lord Corporation, Erie, Pa., is applied on the supporting base layer via spray coating, and then the top layer is coated as described in Example I.

60 The resulting three-layer film on the glass substrate was then immersed into water overnight, about 23 hours, and the freestanding film was released from the glass automatically resulting in a three-layer intermediate transfer member with a 80 micron thick polyaniline/polyimide base layer with a ratio by weight of 15/85; a 100 nanometer thick adhesive layer 65 thereover; and a 20 micron thick polyaniline/polyetherimide-b-polysiloxane top layer with a copolymer ratio by weight of 10/90.

## 15

## Surface Resistivity Measurement

The above ITB members or devices of Comparative Example 1 and Example I were measured for surface resistivity (averaging four to six measurements at varying spots, 72° F./65 percent room humidity) using a High Resistivity

## 16

2. An intermediate transfer member in accordance with claim 1 wherein said polyetherimide/polysiloxane is a polyetherimide-b-polysiloxane copolymer.

3. An intermediate transfer member in accordance with claim 2 wherein said polyetherimidepolysiloxane is represented by



Meter (Hiresta-Up MCP-HT450 from Mitsubishi Chemical Corp.), and the surface resistivity results are illustrated in Table 1 below.

TABLE 1

|                       | Surface Resistivity (ohm/sq)     | Contact Angle |
|-----------------------|----------------------------------|---------------|
| Comparative Example 1 | $(4.67 \pm 0.17) \times 10^{11}$ | 51°           |
| Example I             | $(5.35 \pm 0.12) \times 10^{11}$ | 102°          |

## Contact Angle Measurement

The advancing contact angles of water (in deionized water) of the ITB devices of Comparative Example 1 and Example I were measured at ambient temperature (about 23° C.), using the Contact Angle System OCA (Dataphysics Instruments GmbH, model OCA15. At least ten measurements were performed, and their averages are also reported in Table 1.

The disclosed ITB device with a polyetherimide-b-polysiloxane top layer (Example I) was much more hydrophobic (about 50 degrees higher contact angle) than the Comparative Example 1 polyimide ITB device.

D10 polydimethylsiloxane refers, for example, to a decamer of a siloxane —Si(CH<sub>3</sub>)<sub>2</sub>—O—, which in turn is a specific example of a ULETRM material selected.

The claims, as originally presented and as they may be amended, encompass variations, alternatives, modifications, improvements, equivalents, and substantial equivalents of the embodiments and teachings disclosed herein, including those that are presently unforeseen or unappreciated, and that, for example, may arise from applicants/patentees and others. Unless specifically recited in a claim, steps or components of claims should not be implied or imported from the specification or any other claims as to any particular order, number, position, size, shape, angle, color, or material.

What is claimed is:

1. An intermediate transfer member comprised of a polyimide substrate, and thereover a polyetherimide/polysiloxane.

4. An intermediate transfer member in accordance with claim 2 wherein said copolymer is prepared by reacting 2,2-bis(2,3-dicarboxyphenoxyphenol)propane dianhydride, metaphenylidiamine, and an aminopropyl-terminated polydimethylsiloxane.

5. An intermediate transfer member in accordance with claim 2 wherein said polyetherimide-b-polysiloxane copolymer is formed by reacting pyromellitic acid with diamino-diphenylether and an aminopropyl-terminated polydimethylsiloxane; reacting biphenyltetracarboxylic acid and pyromellitic acid with p-phenylenediamine, diaminodiphenylether, and an aminopropyl-terminated polydimethylsiloxane;

40 or by reacting pyromellitic dianhydride and a benzophenone tetracarboxylic dianhydride copolymeric acid with 2,2-bis[4-(8-aminophenoxy)phenoxy]-hexafluoropropane, and an aminopropyl-terminated polydimethylsiloxane.

45 6. An intermediate transfer member in accordance with claim 2 wherein said copolymer possesses a weight average molecular weight of from about 5,000 to about 1,000,000.

7. An intermediate transfer member in accordance with claim 2 wherein said copolymer possesses a weight average molecular weight of from about 20,000 to about 200,000.

8. An intermediate transfer member in accordance with claim 1 wherein said polyetherimide/polysiloxane is a copolymer or a block copolymer.

55 9. An intermediate transfer member in accordance with claim 1 wherein the weight percent of said polysiloxane in said polyetherimide/polysiloxane is from about 10 to about 50 weight percent.

10. An intermediate transfer member in accordance with claim 1 wherein said polyimide is at least one of polyimide, polyetherimide, polyamidimide polyetherimide/polysiloxane, or mixtures thereof.

60 11. An intermediate transfer member in accordance with claim 1 wherein said member is a weldable belt.

12. An intermediate transfer member in accordance with claim 1 wherein said polyetherimide/polysiloxane is con-

17

tained in a layer over said polyimide substrate, and said layer further comprises a second polymer selected from the group consisting of a polyimide, a polycarbonate, a polyamidimide, a polyphenylene sulfide, a polyamide, a polysulfone, a polyetherimide, a polyester, a polyvinylidene fluoride, a polyethylene-co-polytetrafluoroethylene, and mixtures thereof, present in an amount of from about 70 to about 90 weight percent based on the weight of total solids.

13. An intermediate transfer member in accordance with claim 1 wherein said member has a surface resistivity of from about  $10^7$  to about  $10^{13}$  ohm/sq.

18

22. An intermediate transfer member in accordance with claim 21 wherein said adhesive layer is of a thickness of from about 1 to about 100 nanometers, and said layer is comprised of an epoxy, a urethane, a silicone, or a polyester.

23. An intermediate transfer belt comprised of a polyimide substrate layer, and thereover a layer comprised of a polyetherimide/polysiloxane copolymer; wherein at least one of said substrate layer and said copolymer layer further contains 10 a conductive component, and wherein said polyetherimide-polysiloxane copolymer is represented by



14. An intermediate transfer member in accordance with claim 13 wherein said surface resistivity is from about  $10^8$  to about  $10^{12}$  ohm/sq.

15. An intermediate transfer member in accordance with claim 1 further comprising an outer release layer positioned 40 on said polyetherimide/polysiloxane.

16. An intermediate transfer member in accordance with claim 15 wherein said release layer comprises a poly(vinyl chloride), a fluorinated ethylene propylene copolymer, a polytetrafluoroethylene, a polyfluoroalkoxy polytetrafluoroethylene, a fluorosilicone, a polymer of vinylidenefluoride, hexafluoropropylene and tetrafluoroethylene, or mixtures thereof.

17. An intermediate transfer member in accordance with claim 1 further including in the polyetherimide/polysiloxane, a conductive component, present in an amount of from about 1 to about 40 percent by weight based on the weight of total solids, and wherein said polyetherimide/polysiloxane is in the form of a layer in continuous contact with said substrate.

18. An intermediate transfer member in accordance with claim 17 wherein said conductive component is a carbon black, a polyaniline, or a metal oxide, present in an amount of from about 3 to about 25 percent by weight based on the weight of total solids.

19. An intermediate transfer member in accordance with claim 1 wherein said member has a surface resistivity of from about  $10^9$  to about  $10^{13}$  ohm/sq.

20. An intermediate transfer member in accordance with claim 19 wherein said surface resistivity is from about  $10^{10}$  to about  $10^{12}$  ohm/sq.

21. An intermediate transfer member in accordance with claim 1 further including an adhesive layer situated between the substrate and the polyetherimide/polysiloxane.

35 wherein said substrate is of a thickness of from about 70 to about 125 microns, and said polyetherimide-b-polysiloxane copolymer in the form of a layer is of a thickness of from about 5 to about 15 microns, and said polyetherimide-b-polysiloxane copolymer possesses a weight average molecular weight of from about 100,000 to about 200,000, and wherein the weight percent thereof of said polysiloxane in said copolymer is from about 20 to about 75, and wherein the total of said components in said copolymer layer is about 100 percent.

24. An intermediate transfer belt in accordance with claim 23 comprising an outer release layer positioned on said polyetherimide/polysiloxane copolymer layer.

25. An intermediate transfer member in accordance with claim 24 wherein said release layer comprises a poly(vinyl chloride), a fluorinated ethylene propylene copolymer, a polytetrafluoroethylene, a polyfluoroalkoxy polytetrafluoroethylene, a fluorosilicone, a polymer of vinylidenefluoride, hexafluoropropylene, and tetrafluoroethylene, or mixtures thereof.

26. A transfer media comprised of a polyimide first supporting substrate layer, and thereover a second layer comprised of a polyetherimide-block-polysiloxane copolymer; an adhesive layer situated between said first layer and said second layer, and wherein at least one of said first layer and said second layer further contain a conductive component.

27. A transfer media in accordance with claim 26 wherein said polyetherimide-polysiloxane block copolymer is represented by

19

20



and wherein said conductive component is polyaniline, carbon black, or mixtures thereof, and a release layer in contact with said second layer, and which release layer is selected from the group consisting of a poly(vinyl chloride), a fluorinated ethylene propylene copolymer, a polytetrafluoroethylene, a polyfluoroalkoxy polytetrafluoroethylene, a fluorosilicone, a vinylidenefluoride, and a hexafluoropropylene tetrafluoroethylene polymer.

**28.** A transfer media in accordance with claim **26** wherein said second layer contains carbon black.

**29.** A transfer media in accordance with claim **26** wherein said substrate is of a thickness of from about 30 to about 200 microns, said adhesive layer is of a thickness of from about 1 to about 75 nanometers, and said polyetherimide-b-polysi-

loxane copolymer in the form of a layer is of a thickness of from about 1 to about 30 microns, and said polyetherimide-b-polysiloxane copolymer possesses a weight average molecular weight of from about 50,000 to about 300,000, and wherein the weight percent thereof of polysiloxane in said copolymer is from about 5 to about 95, and wherein the total of the components in said copolymer layer is about 100 percent.

**30.** A belt in accordance with claim **23** which belt functions to permit the transfer of a xerographic developed image from a photoconductor to said belt, and thereafter transferring from said belt said image to paper.

\* \* \* \* \*